

# UNITED STATES PATENT OFFICE.

MARIUS RATIGNIER, OF LYON, FRANCE.

## TREATMENT OF OPEN-MESH TEXTILE FABRICS.

Specification of Letters Patent. Patented Mar. 23, 1915.

1,133,062.

No Drawing.

Application filed April 21, 1913. Serial No. 762,704.

To all whom it may concern:

Be it known that I, MARIUS RATIGNIER, a citizen of France, residing at 56 Cours Morand, Lyon, France, have invented new and useful Improvements in the Treatment of Open-Mesh Textile Fabrics, of which the following is a specification.

This invention relates to treatment of open mesh textile fabrics; and it comprises 10 a process of waterproofing and sizing malines, tulles, nets and other textile fabrics of the open mesh type, wherein such fabric is treated with a solution of nitrocellulose in a solvent containing sufficient amyl acetate to 15 retard the speed of drying, and is thereafter dried with relative slowness; all as more fully hereinafter described and as claimed.

Open mesh fabrics, such as tulles, nets, and the like, are used in large quantities by 20 modistes and milliners for trimming and decorating women's apparel, being made up, for example, in the form of bows, pompons, ruchings, etc., for dresses and hats. Sometimes entire hats are made from such fabrics. 25 It is of the utmost importance therefore that the goods thus made up shall retain the shape given them, the artistic effect and stylish appearance of such decorations being due largely to the skill of the modiste or milliner 30 in producing the particular design of trimming in question. Unfortunately, however, fabrics of this kind have in themselves little or no body or shape-retaining properties, owing chiefly to the fact that they are of 35 such open texture and are composed usually of rather fine threads. It is therefore necessary to stiffen these fabrics in some way, as by sizing, in order to give the forms into which they are shaped even a moderate degree 40 of permanence. But simple sizing is at best a makeshift since these fabrics are very sensitive to moisture and readily soften and lose shape in humid atmosphere.

It has been attempted heretofore to stiffen 45 and at the same time to render waterproof open mesh fabrics of the type here in question by applying to them various solutions containing water proofing agents. These attempts have not been wholly satisfactory, 50 however, the protective coating thus placed on the threads being invariably more or less brittle and non-adherent, and also rendering the fabric too heavy and stiff. Too much stiffening is as undesirable as too little. The 55 peculiar characteristics of tulles, nets, etc., which sharply distinguish them from ordi-

nary fabrics, have rendered their successful treatment a difficult problem.

I have found that the unsatisfactory results obtained heretofore in attempting to 60 waterproof open-mesh fabrics have been due for the most part to improper methods of applying the waterproofing agents to the goods. The solvents employed in the solutions were allowed to dry too rapidly after 65 application, with the result either that there was insufficient impregnation of the threads to afford good anchorage for the coating left after evaporation, or else that too thick a 70 coating was left. In the first case, the coating was brittle and non-adherent to such an extent that it scaled off and soon ceased to protect the goods; while in the second case, not only did the goods lose their delicate 75 sheerness by over-weighting and over-stiffening, but their texture was apt to be more or less distorted and warped by the shrinkage of the excessively thick layers of waterproofing materials upon rapidly drying.

According to the process of the present 80 invention, the difficulties above pointed out are avoided and new advantages gained. Permanently waterproof tulle and the like are obtained having just the desired amount of stiffness and possessing particularly fine 85 luster and feel. Open mesh fabrics treated by the new method do not soften when exposed to moisture and always retain the shape given them.

My new process consists in applying to 90 fabrics of the class described a liquid composition comprising a cellulose ester, such as a nitrocellulose, dissolved in a suitable solvent, and in retarding the evaporation of the solvent after application of the composition, by using in the composition an evaporation retarder which is itself advantageously a solvent of the ester or mixture of esters employed. The nitrocellulose may be 95 in the form of collodion, gun cotton, celluloid, or derivatives of any of these, dissolved in any of their usual solvents such as alcohol and ether, or the like. To a solution of any of these is added amyl acetate in proportions varying with the nature of the particular fabric to be treated. The amyl acetate, by reason of its higher boiling point and slower rate of evaporation, serves to retard the evaporation of the other and more volatile solvents mentioned, thus permitting thorough permeation of the fabric threads by the liquid composition and en-

abling the formation of a very thin protective sheath or envelop of waterproofing agent incasing each thread and firmly locked thereto. The amount of amyl acetate used depends upon the degree of retardation desired in a given instance. It is very advantageous also to incorporate such a material as gum lac in the liquid coating composition, since the toughness and adherence of the final dried coating are thereby enhanced.

10 The fabrics may be easily impregnated with the mixture described in any suitable way, as for example by means of apparatus commonly used in dressing fabrics.

15 In a typical embodiment of the invention I may employ a mixture suitable particularly for the treatment of black fabrics and prepared as follows: Three kilograms of 20 gum-lac are dissolved in two liters of alcohol, to which is added eight liters of amyl acetate, the whole being then mixed with six and a half liters of collodion and tinted with black. This solution has the property 25 of imparting not only impermeability to the fabric but also an excellent surface, an exceptionally brilliant gloss, and absolute fastness of color. The solution having been ap-

plied to the fabric, drying is allowed to occur slowly, thus insuring complete permeation of the fabric threads by the mixture with consequent locking thereto of the residual protective coating left after evaporation of the solvents is finally complete.

30 What I claim is:

1. The process of impregnating and waterproofing open mesh fabrics such as tulle and the like which comprises treating such a fabric with a solution comprising collodion, gum lac, and amyl acetate, and allowing the treated fabric to dry slowly.

2. The process of impregnating and waterproofing open mesh fabrics such as tulle and the like which comprises treating such a fabric with a solution comprising collodion, 45 gum lac, and amyl acetate, in the approximate ratio of 3 parts by weight of gum lac dissolved in alcohol, 8 parts by volume of amyl acetate and 6.5 parts by volume of collodion and allowing the treated fabric to 50 dry slowly.

35 MARIUS RATIGNIER.

Witnesses:

GASTON YEAUNIAUX,  
MARIUS HERMAZ.